# EUROPEAN PATENT SPECIFICATION

(11) **EP 0 354 775 B1**
(45) Date of publication and mention of the grant of the patent: **27.04.1994**
(21) Application number: 89308081.2
(22) Date of filing: 09.08.1989
(51) Int. Cl.: B24B 9/16, B24B 37/04, B24D 7/02

(54) **Diamond tool**
Diamantwerkzeug
Outil diamanté

(30) Priority: 10.08.1988 ZA 885879
(43) Date of publication of application: 14.02.1990
(73) Proprietor: DE BEERS INDUSTRIAL DIAMOND DIVISION (PROPRIETARY) LIMITED, Johannesburg, Transvaal (ZA)
(72) Inventor: Burns, Robert Charles, Johannesburg Transvaal (ZA); Tolkowsky, Gabriel Shraga, Antwerpen (BE); Cronselaar, Gerrit Jan Lucas, No. 2 Nijlen (BE); Phaal, Cornelius, Bagshot Surrey, GU19 5EF (GB)
(74) Representative: Jones, Alan John

(56) References cited:
- BE-A- 775 418
- DE-A- 3 032 027
- FR-A- 993 724
- GB-A- 1 161 885
- GB-A- 2 158 086
- SU-A- 878 551
- US-A- 2 863 750
- SOVIET INVENTIONS ILLUSTRATED Derwent Publications Ltd. abstract number 82-75992E 36 Bul.41/7.11.81

## Description

This invention relates to diamond scaifes.

A diamond scaife is a tool which comprises a cast iron plate, one surface of which has a paste containing a plurality of small diamond particles uniformly spread across it. The paste is rubbed on to the surface and then worked in with a piece of low quality diamond. A diamond scaife is a tool used for polishing diamond.

US-A-2 863 750 discloses a method of mechanically setting diamond particles in, and renewing the solid working surface of, a metal diamond-abrasive wheel, consisting essentially of the steps: applying a mixture comprising diamond particles, glass particles of larger size than said diamond particles and a carrier selected from the group consisting of petroleum jelly and a heavy grease, to the working surface of said wheel; rotating said wheel at a speed in excess of about 300 rpm; urging a freely rotatable roller against said working surface while said wheel is rotating under a pressure sufficient to cause said glass particles to cut said working surface of said wheel and to loosen previously set diamond particles in said working surface; and thereafter urging said roller against said working surface while the wheel is rotating under a pressure sufficient to crush said glass particles to a size smaller than said diamond particles and to force said diamond particles into the interstices of said working surface.

### SUMMARY OF THE INVENTION

The present invention provides a diamond scaife comprising an iron-based working surface having a bonding paste of an organic binder uniformly spread across it, the paste containing a plurality of particles of single crystal and polycrystalline diamond which are partially embedded in the iron-based working surface.

According to another aspect of the invention, there is provided a method of making a diamond scaife as described above which includes the steps of providing an iron-based working surface, depositing a layer of a bonding paste of an organic binder on the surface, the bonding paste containing a plurality of single crystal and polycrystalline diamond particles, and causing the diamond particles to become partially embedded in the working surface.

### DESCRIPTION OF THE DRAWING

Figure 1 illustrates a perspective view of a diamond scaife of the invention; and
Figure 2 illustrates a section through the diamond scaife during the course of its manufacture.

### DESCRIPTION OF EMBODIMENTS

The abrasive elements for the diamond scaife will be constituted by a mixture of single crystal and polycrystalline diamond. The paste will constitute a thin film across the iron-based working surface and is believed, in use, to perform some lubricating function. The paste will contain the diamond particles which will also be partially embedded in the iron-based working surface. It has been found that use of this scaife results in polishing being achieved without the metal surface coming into contact with the diamond or other material being polished.

The working surface may be made of any suitable iron-based material, but is preferably cast iron.

The paste will have a coherency sufficient to allow it to remain on the working surface without flowing off it. It will act, at least in part, to locate the diamond particles on the working surface and also as a lubricant. The paste is constituted by an organic binder which may be any known in the art. Examples of suitable binders include cellulose ethers and esters, phenolic resins, dextrin and other similar materials. One preferred organic binder is methyl cellulose.

The diamond particles will be fine, i.e. they will generally have a particle size of 40 microns or less. When the diamond scaife is to be used for a relatively rough polishing operation, the diamond particles will typically have a size of 10 to 40 microns. For smoothing operations, finer diamond particles of the order of 2 to 10 microns will be used.

The diamond particles will be made up of a combination of single crystal diamond and polycrystalline diamond. The polycrystalline diamond particles will generally be produced by crushing a diamond compact. The diamond compact may be one which contains a solvent second phase such as that described in United States Patent No. 3,745,623 and British Patent No. 1,489,130. The polycrystalline diamond may also be produced from a thermally stable diamond compact, that is a diamond compact which can withstand a temperature of 1200°C in a vacuum, inert or non-oxidising atmosphere without any significant graphitisation of the diamond occurring. Examples of such compacts are described in United States Patents Nos. 4,224,380, 4,534,773 and British Patent No. 2,158,086. It is preferred that the polycrystalline diamond is thermally stable, particularly of the type described in British Patent No. 2,158,086.

The diamond scaife may be made by a method which forms another aspect of the invention. As described above, this method involves providing an iron-based working surface, depositing a layer of a bonding paste of an organic binder on the surface, the bonding paste containing a plurality of single crystal and polycrystalline diamond particles, and causing the diamond particles to become partially embedded in the working surface. Generally, the diamond particles will be caused to become partially embedded in the working surface by rotating that surface and bringing the rotating surface into contact with a diamond surface which is generally a piece of low quality diamond.

The bonding paste will preferably be deposited on the working surface in the form of a liquid which contains a solvent and the solvent then allowed to evaporate at least partially, to produce the coherent paste. The solvent will vary according to the nature of the organic binder. Preferably the organic binder will be such that the solvent is water.

Generally, two layers of the bonding paste will be deposited on the surface, one on top of the other, the layer adjacent the working surface containing the polycrystalline diamond particles and the other layer containing the single crystal diamond particles. In this form of the invention, the single crystal diamond particles may be smaller than the polycrystalline diamond particles so that when the particles are caused to become partially embedded in the working surface, the fine single crystal diamond particles tend to locate in spaces between the polycrystalline diamond particles.

An embodiment of the invention will now be described with reference to the accompanying drawings. Referring to Figure 1 of this drawing, there is shown a cast-iron disc 10 of a diamond scaife which has an upper working surface 12. This working surface 12 has a uniform layer of bonding paste of an organic binder uniformly spread across it. This bonding paste includes a plurality of diamond particles 14 evenly distributed through it and partially embedded in the working surface 12 of the disc 10.

The diamond scaife may be made by depositing a first layer 16 on the working surface 12 of the disc 10 - see Figure 2. This layer 16 will consist of an organic binder containing a plurality of the polycrystalline diamond particles. On the layer 16 there is deposited a second layer 18 of an organic binder containing a plurality of the single crystal diamond particles. The layers 16 and 18 are each deposited by providing a liquid mixture of the organic binder, a suitable solvent and the diamond particles, applying that liquid mixture to the relevant surface and allowing the solvent to evaporate leaving a coherent paste layer. The diamonds of the two layers are worked into the surface 12 by rotating the disc 10, for example at a speed of about 2000rpm, and bringing that rotating surface into contact with a diamond surface such as that provided by a low quality diamond. The resulting product is that illustrated by Figure 1.

In a particular example of the invention, one carat of crushed thermally stable diamond compact containing a silicon second phase (as described in British Patent No. 2,158,086) and of particle size less than 40 microns was rubbed on the cast iron working surface of a scaife with a binder such as dextrin or phenolic resin in a solvent. The solvent was allowed to evaporate leaving a coherent paste. A paste of fine single crystal diamond particles in water containing methyl cellulose was then applied to the coated surface. The water was allowed to evaporate leaving a thin film or layer of coherent methyl cellulose paste containing the diamond particles. The coated working surface was then rotated at a speed of 2000rpm and brought into contact with a low quality diamond. This contact was maintained for 75 minutes to work the polycrystalline diamond particles and the single crystal diamond particles into the working surface. It was found that diamond polishing could be achieved with this scaife without the metal surface coming into contact with the diamond being polished. Further, improved cutting performance was experienced in relation to diamond of 2 carats or larger. This makes the diamond scaife ideally suited for working stressed diamonds.

## Claims

1. A diamond scaife comprising an iron-based working surface (12) having a bonding paste of an organic binder uniformly spread across it, the paste containing a plurality of particles (14) of single crystal and polycrystalline diamond which are partially embedded in the iron-based working surface (12).

2. A diamond scaife according to claim 1 wherein the organic binder is selected from phenolic resins, cellulose ethers and esters and mixtures thereof.

3. A diamond scaife according to claim 1 or claim 2 wherein the working surface (12) is a cast iron working surface.

4. A diamond scaife according to any one of the preceding claims wherein the polycrystalline diamond particles (14) are thermally stable polycrystalline diamond particles.

5. A diamond scaife according to any one of the preceding claims wherein the diamond particles (14) have a size of 40 microns or less.

6. A method of making a diamond scaife according to any one of the preceding claims including the steps of providing an iron-based working surface (12), depositing a layer of a bonding paste of an organic binder on the surface, the bonding paste containing a plurality of single crystal and polycrystalline diamond particles (14), and causing the diamond particles to become partially embedded in the working surface (12).

7. A method according to claim 6 wherein the bonding paste is deposited in the form of a liquid containing a solvent and the solvent is allowed to evaporate, at least partially, to produce the paste.

8. A method according to claim 7 wherein the solvent is water.

9. A method according to claim 7 or claim 8 wherein two layers of bonding paste are applied to the surface (12), one on top of the other, the layer (16) adjacent the working surface containing the polycrystalline diamond particles and the other layer (18) containing the single crystal diamond particles.

10. A method according to any one of claims 6 to 9 wherein the diamond particles are caused to become partially embedded in the working surface (12) by rotating that surface (12) and bringing the rotating surface (12) into contact with a diamond surface.

## Patentansprüche

1. Diamantpolierwerkzeug mit einer auf Eisen basierenden Arbeitsoberfläche (12), über welche eine Haft- bzw. Bindepaste aus einem organischen Bindemittel gleichförmig verteilt ist, wobei die Paste eine Vielzahl von Partikeln (14) aus Einkristall- und polykristallinen Diamanten enthält, welche in die auf Eisen basierende Arbeitsoberfläche (12) teilweise eingebettet sind.

2. Diamantpolierwerkzeug gemäß Anspruch 1, wobei das organische Bindemittel aus phenolischen Harzen, Zelluloseethern und -estern und Mischungen hiervon ausgewählt ist.

3. Diamantpolierwerkzeug gemäß Anspruch 1 oder 2, wobei die Arbeitsoberfläche (12) eine gußeiserne Arbeitsoberfläche ist.

4. Diamantpolierwerkzeug gemäß einem der vorhergehenden Ansprüche, wobei die polykristallinen Diamantpartikel (14) thermisch stabile polykristalline Diamantpartikel sind.

5. Diamantpolierwerkzeug gemäß einem der vorhergehenden Ansprüche, wobei die Diamantpartikel (14) eine Größe von 40 µm oder weniger aufweisen.

6. Verfahren zum Herstellen eines Diamantpolierwerkzeuges gemäß einem der vorhergehenden Ansprüche, mit den Schritten, eine auf Eisen basierende Arbeitsoberfläche (12) vorzusehen, eine Schicht aus einer Haft- bzw. Bindepaste aus einem organischen Bindemittel auf der Oberfläche abzuscheiden, wobei die Bindepaste eine Vielzahl von Einkristall- und polykristallinen Diamantpartikeln (14) enthält, und zu veranlassen, daß die Diamantpartikel in die Arbeitsoberfläche (12) teilweise eingebettet werden.

7. Verfahren gemäß Anspruch 6, wobei die Bindepaste in der Form einer Flüssigkeit mit einem Lösungsmittel abgeschieden wird und wobei man das Lösungsmittel zumindest teilweise evaporieren läßt, um die Paste zu erzeugen.

8. Verfahren gemäß Anspruch 7, wobei das Lösungsmittel Wasser ist.

9. Verfahren gemäß Anspruch 7 oder Anspruch 8, wobei zwei Schichten von Bindepaste auf die Fläche (12) aufgebracht werden, und zwar eine über der anderen, wobei die Schicht (16) benachbart der Arbeitsoberfläche die polykristallinen Diamantpartikel enthält und die andere Schicht (18) die Einkristall-Diamantpartikel enthält.

10. Verfahren gemäß einem der Ansprüche 6 bis 9, wobei veranlaßt wird, daß die Diamantpartikel in die Arbeitsoberfläche (12) teilweise eingebettet werden, indem jene Fläche (12) in Drehung versetzt wird und die sich drehende Fläche (12) in Kontakt mit einer Diamantoberfläche gebracht wird.

## Revendications

1. Disque de polissage de diamant (scaife) comprenant une surface d'usinage à base de fer (12) ayant une pâte de liage d'un liant organique uniformément répandue sur elle, la pâte contenant une pluralité de particules (14) de diamant monocristallin ou polycristallin qui sont partiellement incrustées dans la surface d'usinage à base de fer (12).

2. Disque de polissage de diamant selon la revendication 1, dans lequel le liant organique est choisi parmi les matériaux suivants: résines phénoliques, éthers cellulosiques et esters de cellulose et mélanges de ces matériaux.

3. Disque de polissage de diamant selon la revendication 1 ou la revendication 2, dans lequel la surface d'usinage (12) est une surface d'usinage en fonte.

4. Disque de polissage de diamant selon l'une quelconque des revendications précédentes, dans lequel les particules de diamant polycristallin (14) sont des particules de diamant polycristallin thermiquement stables.

5. Disque de polissage de diamant selon l'une quelconque des revendications précédentes, dans lequel les particules de diamant (14) ont une dimension de 40 microns ou moins.

6. Procédé de fabrication d'un disque de polissage de diamant selon l'une quelconque des revendications précédentes, comprenant les étapes consistant à fournir une surface d'usinage à base de fer (12), déposer une couche de pâte de liage d'un liant organique sur la surface, la pâte de liage contenant une pluralité de particules de diamant monocristallin et polycristallin (14), et faire s'incruster partiellement les particules de diamant dans la surface d'usinage (12).

7. Procédé selon la revendication 6, dans lequel la pâte de liage est déposée sous la forme d'un liquide contenant un solvant et dans lequel on fait évaporer le solvant au moins partiellement, pour produire la pâte.

8. Procédé selon la revendication 7, dans lequel le solvant est de l'eau.

9. Procédé selon la revendication 7 ou la revendication 8, dans lequel deux couches de pâte de liage sont appliquées sur la surface (12), l'une par-dessus l'autre, la couche (16) adjacente à la surface d'usinage contenant les particules de diamant polycristallin et l'autre couche (18) contenant les particules de diamant monocristallin.

10. Procédé selon l'une quelconque des revendications 6 à 9, dans lequel on fait s'incruster partiellement les particules de diamant dans la surface d'usinage (12) en faisant tourner cette surface (12) et en mettant la surface en rotation (12) en contact avec une surface de diamant.
